

1

3,294,696

**DRY CLEANING PROCESS AND COMPOSITIONS**  
 Maurice Goharel, Saint-Auban, Basses-Alpes, Laurent Seigneurin, Salindres, Gard, France, and Lucien Hamelin (by France Hamelin, executrix for the estate of Lucien Hamelin), Vanves, Seine, France, assignors to Produits Chimiques Pechiney-Saint-Gobain, Neuilly-sur-Seine, France  
 No Drawing. Filed May 18, 1964, Ser. No. 368,367  
 Claims priority, application France, May 20, 1963,  
 935,401  
 3 Claims. (Cl. 252—172)

This invention relates to the art of dry cleaning and more particularly to a dry cleaning process which makes use of a new and improved dry cleaning agent.

Among the well known dry cleaning solvents, present use is made principally of tetrachlorethylene and trichloroethylene as representative. These solvents have relatively high boiling points, such that in a normal cleaning cycle, which includes the following main steps of washing, wringing, drying and deodorizing, the drying and deodorizing steps consume a considerable amount of time.

Dichloroethylene has also been proposed for use in dry cleaning. However, dichloroethylene attacks certain synthetic and artificial materials formed into textile fibers and particularly fibers formed of cellulose acetate and vinyl resins. Furthermore, dichloroethylene is not entirely non-inflammable and thus does not meet the safety requirements.

Certain chlorofluorinated hydrocarbon derivatives formed of one or two carbon atoms and having as many fluorine atoms as carbon atoms have also been proposed. However, they present the deficiency in that their boiling points are too low. In order to use them for dry cleaning, it is necessary to make use of special machines adapted for use with such volatile solvents, and even with such specific devices, the losses which may take place during the cleaning cycle or in the storage and handling of the solvent are excessive.

It is an object of this invention to provide a dry cleaning process which makes use of a dry cleaning agent that overcomes the deficiencies heretofore described and where the dry cleaning agent is non-inflammable, is capable of being easily distilled, does not have too low a boiling point and does not have any undesirable effects on the textile fibers formed of synthetic or artificial resins.

In accordance with the practice of this invention, the dry cleaning process makes use of a new and improved dry cleaning agent consisting of a liquid composition composed essentially of hexafluorodichlorobutene or of a liquid composition containing hexafluorodichlorobutene as an essential and major ingredient. The term "hexafluorodichlorobutene" means a compound having the formula  $C_4F_6Cl_2$  and which may comprise a mixture of one or more of its isomers and particularly



With the composition containing hexafluorodichlorobutene, use can be made of one or more other compounds in combination therewith selected from the group of solvents consisting of aliphatic hydrocarbon halogenated derivatives having a boiling point close to that of hexafluorodichlorobutene, such for example as a halogenated aliphatic hydrocarbon derivative having a boiling point which does not deviate from the boiling point of hexafluorodichlorobutene by more than 25° to 30° C. and preferably by not more than 15° C.

2

The proportions of the constituents of said composition are selected so as to maintain, and preferably to improve, the required properties for use in dry cleaning purposes. Thus during the distillation or re-distillation of such compositions, the initial proportions of the constituents will be maintained.

In addition to its non-inflammability, hexafluorodichlorobutene is characterized by being chemically stable, having a solvent power sufficiently high without having a tendency to attack the textile fibers or the buttons or plastic ornaments which are on the garments and it is also free from odor.

In accordance with the practice of this invention, adjuvants can be incorporated in the usual small proportions with the hexafluorodichlorobutene composition. Such adjuvants may be illustrated by the non-ionic, cationic or anionic tensio-active agents, reinforcing cleaning agents generally employed in the dry cleaning systems and in which such adjuvants preferably are selected to be compatible in the composition.

The compositions described find use also as a solvent for cleaning or for degreasing in general and particularly for the cleaning of devices fabricated of metals and insulating materials such as employed in electric and telephone apparatus, motors, and the like.

It is also an object of this invention to provide a dry cleaning process which includes the step of washing the textile fibers and other garments by means of a liquid formed essentially of hexafluorodichlorobutene or in which hexafluorodichlorobutene is an essential and major ingredient.

The following examples are given by way of illustration, but not by way of limitation, of this invention.

## EXAMPLES 1 TO 6

35 In a test for attack by hexafluorodichlorobutene, different textile fabrics made of cellulose triacetate, polyvinyl chloride, polyamide 11, polyamide 6/6, polyacrylonitrile and glycol polyterephthalate were immersed in hexafluorodichlorobutene using 15 volumes of the hexafluorodichlorobutene per part by weight of the fabric.

Textile fabrics made of cellulose triacetate and polyvinyl chloride are known to be particularly sensitive to the action of organic solvents. For both of these fabrics, the fabrics were tested by immersion in hexafluorodichlorobutene for ½ hour at 20° C., for ½ hour at 30° C. and for 4 hours at boiling point temperature using hexafluorodichlorobutene under reflux in a Soxhlet extractor. The results are set forth in the following Table I.

50 For fabric materials other than formed of cellulose triacetate and polyvinyl chloride, the attack tests were carried out in a Soxhlet extractor at the boiling point temperature of the hexafluorodichlorobutene with exposure for 30 minutes.

In parallel tests, made for comparative purposes, the identical tests were carried out on identical fabrics in which trichloroethylene and tetrachloroethylene were used instead of the hexafluorodichlorobutene. After treatment, the fabrics were dried and the following measurements were made:

55 (1) Dimensional stability calculated as shrinkage or lengthening warp-wise as well as weft-wise of the fibers.  
 (2) Resistivity of the fabric to splitting.

In the following tables, the results of the tests are indicated. They are expressed in percent variation with respect to the untreated reference material. The values marked with the minus sign indicate shrinkage of the fabric sample while the plus sign indicates lengthening.

Table I

| Nature of fabric samples | Conditions of treatment of fabric samples    | Solvent                | Dimensional stability in percent         |            | Resistance to bursting tests in percent |
|--------------------------|----------------------------------------------|------------------------|------------------------------------------|------------|-----------------------------------------|
|                          |                                              |                        | Warp                                     | Weft       |                                         |
| Polyvinyl chloride       | 20° C. during 1/2 an hour                    | {HFDB<br>TCE           | 0<br>-30                                 | 0<br>22.5  | -2.9                                    |
|                          | 30° C. during 1/2 an hour                    | {HFDB<br>PCE           | 0<br>-0.25                               | 0<br>-0.25 | +2<br>+3.4                              |
|                          | Boiling during 4 hours in Soxhlet apparatus. | {HFDB<br>TCE or<br>PCE | 0<br>Attacked, becomes hard and brittle. | -0.5       | -2.9                                    |
| Cellulosic triacetate    | 20° C. during 1/2 an hour                    | {HFDB<br>PCE           | 0<br>-5                                  | 0<br>-3.5  | -----                                   |
|                          | Boiling during 4 hours in Soxhlet apparatus. | {HFDB<br>PCE           | -0.75<br>-12                             | -1<br>-3   | -----                                   |

Table II

|                            | Solvent      | Dimensional Stability in percent |             | Resistance to bursting tests in percent |
|----------------------------|--------------|----------------------------------|-------------|-----------------------------------------|
|                            |              | Warp                             | Weft        |                                         |
| Polyamide 11*              | {HFDB<br>PCE | 0<br>-2.25                       | 0<br>-1.25  | +0.9<br>-5.3                            |
| Polyamide 6/6*             | {HFDB<br>PCE | +0.25<br>+0.75                   | +1<br>+1.25 | -5.6<br>-9.9                            |
| Polyacrylonitrile*         | {HFDB<br>PCE | 0<br>-0.75                       | 0<br>-2.25  | +1.2<br>-4                              |
| Glycol polyterephthalate.* | {HFDB<br>PCE | 0<br>-1.75                       | 0<br>-1.5   | +5.9<br>-10.4                           |

\* Treatment of fabric samples during 4 hours at the boiling point in the solvent into the Soxhlet extractor.

#### EXAMPLES 7 TO 10

Resin samples composed of polystyrene and of styrene acrylonitrile copolymers were submitted to the action of hexafluorodichlorobutene for 30 minutes at 20° C. and for 30 minutes at 30° C. Such resins are often used for making buttons and ornaments employed on garments. The weight variation of the samples were determined by comparison to untreated samples.

Identical tests were carried out on the same resins with tetrachloroethylene.

The results are summarized in Table III in which the values having the minus sign indicate a loss in weight by comparison to a reference sample while values having the plus sign indicate swelling of the resin, indicative of attack.

It will be noticed that the hexafluorodichlorobutene is practically free from attack on the resins while the tetrachloroethylene strongly attacks, particularly the polystyrene resins.

Table III

| Species of resin tested         | Solvent      | Change in weight of the samples in percent with respect to the reference blanks |            |
|---------------------------------|--------------|---------------------------------------------------------------------------------|------------|
|                                 |              | 20° C.                                                                          | 30° C.     |
| Polystyrene                     | {HFDB<br>PCE | -0.1<br>-34                                                                     | 0<br>-30.5 |
| Copolymer acrylonitrile styrene | {HFDB<br>PCE | +0.1<br>+0.3                                                                    | 0<br>+2.2  |

When the hexafluorodichlorobutene is employed in combination with other aliphatic halogenated hydrocarbon derivatives, such as difluorodichloroethane it is desirable to limit the amount of dilution so that the hexafluorodichlorobutene will still constitute more than 50% by weight of the composition and preferably more than

70% by weight of the composition. When other adjuvants are employed, it is undesirable to make use of such adjuvants in an amount which will total more than 5% by weight of the composition and preferably less than 2% by weight of the composition. The following will represent dry cleaning compositions which may be employed in the practice of this invention:

#### EXAMPLE A

100% by weight hexafluorodichlorobutene

#### EXAMPLE B

75% by weight hexafluorodichlorobutene

25% by weight difluorodichloroethane

#### EXAMPLE C

78% by weight hexafluorodichlorobutene

20% by weight difluorodichloroethane

1% by weight wetting agent

1% by weight surface active agent

It will be understood that changes may be made in the details of formulation and application without departing from the spirit of the invention, especially as defined in the following claims.

We claim:

1. In a dry cleaning process for products containing some synthetic resinous materials, the step of washing the product with a liquid composition consisting essentially of at least 50 percent by weight hexafluorodichlorobutene as an essential and major ingredient with the remainder being formed essentially of an aliphatic halogenated dry cleaning hydrocarbon having a boiling point within 30° C. of the hexafluorodichlorobutene and which is compatible therewith.

2. In a dry cleaning process, the step of treating the product to be dry cleaned with a liquid composition consisting essentially of hexafluorodichlorobutene.

3. The dry cleaning process as claimed in claim 1 in which the hexafluorodichlorobutene comprises more than 75% by weight of the liquid composition.

#### References Cited by the Examiner

##### UNITED STATES PATENTS

2,436,357 2/1948 Gochenour et al. ---- 260—653.3  
3,042,479 7/1962 Lawrence et al. ---- 252—172 XR

#### OTHER REFERENCES

Lovelace et al.: "Aliphatic Fluorine Compounds," Reinhold Pub. Corp., New York' (1958) (pages 116—117 relied on).

LEON D. ROSDOL, Primary Examiner.

JULIUS GREENWALD, Examiner.

J. T. FEDIGAN, Assistant Examiner.